

## UNITED STATES PATENT OFFICE

JOHN BRUNNER, OF CHICAGO, ILLINOIS

## HEAT TREATMENT OF STEEL RAILS

No Drawing. Original application filed October 22, 1931, Serial No. 570,496. Divided and this application filed June 11, 1932. Serial No. 616,761.

This invention relates to metallurgy and more particularly to the heat treatment of metals and alloys to improve the qualities thereof and still more particularly to the heat treatment of steel rails. This application is a divisional application of application Serial No. 570,496 filed October 22, 1931 entitled "Heat treatment of steel rails".

This invention is substantially an improvement of the invention set forth in my U. S. Patent No. 1,277,372 issued September 3, 1918.

The process of U. S. Patent No. 1,277,372 substantially comprises a method of heat treating steel rails to obtain therein a more uniform and fine grain structure and a better surface than had heretofore been obtainable. The method substantially comprises rolling the rail to a section larger than the desired finished section; cooling the rail to temperatures below the thermal critical range; reheating the rail to temperatures above the thermal critical temperatures (approximately 800° C.); rolling the rail to the desired finished section; and slowly cooling the rail to room temperatures. This method produced a finished rail having a fine grain structure which imparted thereto great toughness. The rail product, however, did not possess sufficient surface hardness to make it resistant to severe service conditions.

One of the objects of the present invention is to increase the surface hardness of the rail product of my prior invention.

Another object of the present invention is to provide heat-treating methods whereby the surface hardness of a steel rail may be materially increased at its ends where the greatest abrasion and battering takes place in service under the rolling loads of motive power and transportation equipment.

Another object of the present invention is to provide a steel rail having an interior of relatively high ductility throughout the entire length of the rail and an exterior of relatively high hardness at the ends of the rail.

Another object of the present invention is to improve and facilitate the manufacture of steel rails.

Other objects and advantages will be ap-

parent as the invention is more fully disclosed.

In accordance with the objects of the present invention I have found that I may impart a relatively high surface hardness to the relatively tough fine grain structure in the rail prepared in accordance with the invention of my prior patent, thereby materially increasing the resistance of the rail to service conditions, by subjecting the rail to certain heat-treating methods. The heat-treating method substantially comprises the following steps:

At the conclusion of the final rolling operation the finished rail is cooled to temperatures approximating 300° C., and is then reheated to relatively uniform temperatures which are slightly above the thermo-critical range of the specific composition of steel used therein and then cooling the head of the rail at and near its ends in a quenching medium until the surface temperature of this part of the rail has been lowered at least partially through the blue-heat range (approximately 288° C. to 316° C.) but to temperatures not lower than 200° C.; thereafter the entire rail is quenched, preferably in oil, to temperatures approximating but not less than about 250° C., and again heated to temperatures above 300° C. but below the thermal critical range for a determined time interval and thereafter cooled slowly in air to atmospheric temperatures.

In this manner I first effect a refinement of the internal grain structure of the rail, increasing its uniformity and toughness, and then a hardening of the surface of the head thereof at and near its ends, thereby obtaining a desired amount of external surface hardness of the rail ends to resist abrasion and battering of the rail ends in the track in service, and a mild hardening of the surfaces intermediate the ends, followed by an annealing or tempering to remove internal stresses and strains incident to the hardening operation.

As a specific embodiment of the practice of this invention I will disclose the method as applied to a steel rail composition comprising carbon .40 to .85%; manganese .40 to 100

1.60%; phosphorus, not over .08%; sulphur, not over .08%; silicon, not over 1.50%, depending on the section of rail used and the intended service of the treated rail.

- 5 In accordance with the teaching of my prior patent a billet of steel in the above noted composition is heated to temperatures above the thermal critical range and rolled into a section approximating but larger than 10 the desired finished rail section and then is cooled to temperatures below the thermal critical range. Preferably but not necessarily the per cent reduction in area remaining is only that which is sufficient to obtain an accurate section of the rail.

The cooled rail is then reheated to relatively uniform temperatures approximating 800° C. and is thereafter rolled to the desired finished section. The finished rail is therefore 20 allowed to cool to an average temperature if not less than 300° C. and is again reheated to relatively uniform temperatures approximating 800° C., and from these temperatures is quenched on the head at and near 25 both ends of the rail until the surface temperatures of this part of the rail has been lowered partially through the blue-heat range but not lower than 200° C. After the ends have been quenched the entire rail is 30 quenched preferably in oil until the surface temperatures of the part of the rail between the pre-quenched ends approximate but are not less than about 250° C. The quenched rail is then transferred into a furnace and 35 heated to minimum temperatures above 300° C. but below the thermal critical range (approximately 600° C.) after a predetermined time interval approximating from one-half to two hours, following which it is allowed 40 to cool slowly in the air to atmospheric temperatures.

The rail product thus produced will be found to have retained the fine grain structure of my prior patent with an exterior surface on top of the head at the end of the rail of greater hardness than heretofore obtainable by cold working means alone. For example, the finished rail product of my prior patent will have a surface hardness of approximately 250-280, as measured on the Brinell scale. The finished rail product of the specific embodiment of the present invention will have a surface hardness of the head at and near the ends of the rail approximating from 340 to 410, depending on the section and intended service of the heat treated rail.

The exact cooling temperatures and the time intervals of cooling may be widely varied depending upon the composition of the steel, the finished hardness desired, and upon the internal grain structure desired in the rail.

While I have disclosed as a specific embodiment the steps of rolling the rail to a section larger than the desired finished section, cool-

ing to below and then reheating to above the thermal critical range, and then rolling to the desired finished section, I may omit this particular sequence of steps and roll the rail directly down to the desired finished section 70 if desired. The rail thus prepared may be cooled to temperatures below the thermal critical range, but above 300° C., reheated to temperatures approximating but above the thermal critical range, and thereafter 75 quenched and otherwise treated as in the specific embodiment described.

Whereas, also the above invention has been disclosed with particularity as regards to its application to a specific rail composition, it 80 is apparent that with modifications in the steel composition, modifications in the heat treating process may be made accordingly. Such modifications and departures are contemplated as may fall within the scope of the 85 following claims:

What I claim is:

1. The method of heat treating steel rails to increase the surface hardness thereof and especially on the head at and near its ends, which comprises heating the rail to temperatures approximating but above the thermal critical range, quenching the head of the rail at and near its ends until the surface temperatures of the head at and near its ends 90 approximate but are not less than 200° C., then quenching the entire rail until the surface temperatures thereof between the pre-quenched ends approximate but are not less than 250° C., reheating the rail to temperatures higher than the quenching temperatures but below the thermal critical temperatures and thereafter slowly cooling to atmospheric 95 temperatures.

2. The method of hardening the surface of steel rails having an approximate composition of carbon .40 to .85%; manganese .40 to 1.60%; phosphorus, not over .08%; sulphur, not over .08%; silicon, not 1.50%; which comprises heating the rail to temperatures approximating but above the thermal critical range, quenching the head of the rail at and near its ends until the surface temperature of the head at and near its ends approximate but are not less than 200° C., then quenching the entire rail until the surface temperatures thereof between the prequenched ends approximate but are not less than 250° C., annealing the rail at temperatures approximating 600° C., and thereafter slowly cooling to 100 room temperatures.

3. The method of hardening the surface of steel rails having an approximate composition of carbon .40 to .85%; manganese .40 to 1.60%; phosphorus, not over .08%; sulphur, not over .08%; silicon, not over 1.50%; which comprises heating the rail to temperatures approximating 800° C., quenching the head of the rail at and near its ends until the surface temperatures of the head at and 105

near its ends approximate but are not less than  $200^{\circ}$  C., then quenching the entire rail until the surface temperatures of the part of the rail between the ends which has not been pre-quenched approximate but are not less than  $250^{\circ}$  C., annealing the rail for a predetermined time interval at temperatures approximating  $600^{\circ}$  C. and thereafter slowly cooling to room temperatures. 5

10 4. The method of hardening the surface of steel rails having an approximate composition of carbon .40 to .85; manganese .40 to 1.60%; phosphorus, not over .08%; sulphur, not over .08%; silicon, not over 1.50%; which comprises heating the rail to temperatures approximating  $800^{\circ}$  C., quenching the head of the rail at and near its ends in water until the surface temperatures of the head at and near its ends approximate but are not less than  $200^{\circ}$  C., then quenching the entire rail until the surface temperatures of the part of the rail between the ends which has not been pre-quenched approximate but are not less than  $250^{\circ}$  C., annealing the rail for a predetermined time interval at temperatures approximating  $600^{\circ}$  C., and thereafter slowly cooling to room temperatures. 15

20 5. The method of forming steel rails which comprises heating the rail ingot or billet to rolling temperatures above the thermal critical range, rolling to a section larger than the desired finished rail section, cooling to temperatures below the thermal critical range, but above about  $300^{\circ}$  C., reheating to temperatures approximating but above the thermal critical range, rolling to the desired finished section, cooling to temperatures below the thermal critical range but above  $300^{\circ}$  C., reheating to temperatures approximating but above the thermal critical range, quenching the head of the rail at and near its ends until the surface temperatures of the head at and near its ends lie within the blue-heat range but above about  $200^{\circ}$  C., then quenching the entire rail until the surface temperatures of the part of the rail between the pre-quenched ends lie within the blue-heat range but above about  $250^{\circ}$  C., annealing the rail at temperatures approximating  $600^{\circ}$  C. for a predetermined time interval, and thereafter slowly cooling to atmospheric temperatures. 25

30 6. The method of forming steel rails having an approximate composition of carbon .40 to .85%; manganese .40 to 1.60%; phosphorus, not over .08%; sulphur, not over .08%; silicon not over 1.50%; which comprises heating the rail ingot or billet to rolling temperatures above the thermal critical range, rolling to a section larger than the desired finished section, cooling to temperatures lower than the thermal critical range, but above about  $300^{\circ}$  C., reheating to temperatures approximating but above the thermal critical range, quenching the head of the rail at and near its ends until the surface temperatures of the head at and near its ends lie within the blue-heat range but above about  $200^{\circ}$  C., then quenching the entire rail until the surface temperatures of the part of the rail between the pre-quenched ends lie within the blue-heat range but above about  $250^{\circ}$  C., annealing the rail at temperatures approximating  $600^{\circ}$  C., and thereafter slowly cooling to atmospheric temperatures. 35

40 7. The method of forming steel rails having an approximate composition of carbon .40 to .85%; manganese .40 to 1.60%; phosphorus, not over .08%; sulphur, not over .08%; silicon, not over 1.50%; which comprises heating the rail ingot or billet to rolling temperatures above the thermal critical range, rolling to a section larger than the desired finished section, cooling to temperatures lower than the thermal critical range, but above about  $300^{\circ}$  C., reheating to temperatures approximating but above the thermal critical range, rolling to the desired finished section, cooling to temperatures below the thermal critical range, but above about  $300^{\circ}$  C., reheating to temperatures approximating but above the thermal critical range, quenching the head of the rail at and near its ends until the surface temperatures of the head at and near its ends lie within the blue-heat range but above about  $200^{\circ}$  C., then quenching the entire rail until the surface temperatures of the part of the rail between the pre-quenched ends lie within the blue-heat range but above about  $250^{\circ}$  C., annealing the rail at temperatures approximating  $600^{\circ}$  C., and thereafter slowly cooling to atmospheric temperatures. 45

50 8. The method of forming steel rails having an approximate composition of carbon .40 to .85%; manganese .40 to 1.60%; phosphorus, not over .08%; sulphur, not over .08%; silicon not over 1.50%; which comprises heating the rail ingot or billet to rolling temperatures above the thermal critical range, rolling to a section larger than the desired finished section, cooling to temperatures lower than the thermal critical range, but above about  $300^{\circ}$  C., reheating to temperatures approximating but above the thermal critical range, quenching the head of the rail at and near its ends until the surface temperatures of the head at and near its ends lie within the blue-heat range but above about  $200^{\circ}$  C., then quenching the entire rail until the surface temperatures of the part of the rail between the pre-quenched ends lie within the blue-heat range but above about  $250^{\circ}$  C., annealing the rail at temperatures approximating  $600^{\circ}$  C., and thereafter slowly cooling to atmospheric temperatures. 55

60 9. The method of forming steel rails having an approximate composition of carbon .40 to .85%; manganese .40 to 1.60%; phosphorus, not over .08%; sulphur, not over .08%; silicon, not over 1.50%; which comprises heating the rail ingot or billet to rolling temperatures above the thermal critical range, rolling to a section larger than the desired finished section, cooling to temperatures lower than the thermal critical range, but above about  $300^{\circ}$  C., reheating to temperatures approximating but above the thermal critical range, quenching the head of the rail at and near its ends until the surface temperatures of the head at and near its ends lie within the blue-heat range but above about  $200^{\circ}$  C., then quenching the entire rail until the surface temperatures of the part of the rail between the pre-quenched ends lie within the blue-heat range but above about  $250^{\circ}$  C., annealing the rail at temperatures approximating  $600^{\circ}$  C., and thereafter slowly cooling to atmospheric temperatures. 65

tween the pre-quenched ends lie within the blue-heat range but above about 250° C., annealing the rail at temperatures approximating 600° C. for approximately one-half to two hours, and thereafter slowly cooling to atmospheric temperatures.

9. The method of forming steel rails which comprises heating a rail ingot or billet to rolling temperatures above the thermal critical range, rolling the rail to the desired finished section, cooling the rail to temperatures below the thermal critical range but above about 300° C., reheating the rail to temperatures approximating but above the thermal critical range, quenching the head of the rail at and near its ends until the surface temperatures of the head at and near its ends approximate but are above 200° C., then quenching the entire rail until the surface temperatures of the part of the rail between the pre-quenched ends approximate but are above 250° C., annealing to temperatures above about 300° C. but below the thermal critical range and thereafter slowly cooling to room temperatures.

10. The method of forming steel rails from a rail ingot or billet having a composition of carbon .40 to .85%; manganese .40 to 1.60%; phosphorus, not over .08%; sulphur, not over .08%; silicon, not over 1.50%; which comprises heating the rail ingot or billet to rolling temperatures above the thermal critical range, rolling the rail to the desired finished section, cooling the rail to temperatures below the thermal critical range but above about 300° C., reheating to temperatures approximating but above the thermal critical range, quenching the head of the rail at and near its ends until the surface temperatures of the head at and near its ends approximate but are above 250° C., then quenching the entire rail until the surface temperatures between the pre-quenched ends approximate but are above 250° C., annealing the rail to temperatures above 300° C. but less than the thermal critical range and thereafter slowly cooling to atmospheric temperatures.

11. The method of forming steel rails from a rail ingot or billet having a composition of carbon .40 to .85%; manganese .40 to 1.60%; phosphorus, not over .08%; sulphur, not over .08%; silicon, not over 1.50%; which comprises heating the rail ingot or billet to rolling temperatures above the thermal critical range, rolling the rail to the desired finished section, cooling the rail to temperatures below the thermal critical range but above about 300° C., reheating to temperatures approximating but above the thermal critical range, quenching the head of the rail at and near its ends until the surface temperatures of the head at and near its ends approximate but are above about 250° C., then quenching the entire rail until the surface temperatures between the pre-quenched ends approximate but

are above 250° C., annealing the rail to temperatures above 300° C., but not less than the thermal critical range for a predetermined time interval and thereafter slowly cooling to atmospheric temperatures.

12. The method of forming steel rails from a rail ingot or billet having a composition approximating carbon .40 to .85%; manganese .40 to 1.60%; phosphorus, not over .08%; sulphur, not over .08%; silicon, not over 1.50%; which comprises heating the rail ingot or billet to rolling temperatures above the thermal critical range, rolling the rail to the desired finished section, cooling the rail to temperatures below the thermal critical range but above about 300° C., reheating to temperatures approximating but above the thermal critical range, quenching the head of the rail at and near its ends until the surface temperatures of the head at and near its ends approximate but are above about 250° C., then quenching the entire rail until the surface temperatures of the rail between the pre-quenched ends approximate but are above about 250° C., annealing the rail to temperatures above 300° C., but less than the thermal critical range for approximately one-half to two hours, and thereafter slowly cooling to atmospheric temperatures.

13. The method of treating steel rails to harden the same which comprises quenching the head of the rail at and near its ends from a temperature above the critical temperature to a temperature approximating but not less than 200° C. and then quenching the entire rail until the surface temperature thereof between the prequenched ends approximate but are not less than 250° C., then reheating the rail to temperatures higher than the quenching temperatures but below the critical temperature and thereafter slowly cooling to room temperatures.

In witness whereof, I have hereunto signed my name.

JOHN BRUNNER. 110

115

120

125

130